

## UNITED STATES PATENT OFFICE.

JOHN C. BAKER, OF NUTLEY, NEW JERSEY.

## BLEACHING PAPER PULP.

No Drawing.

Application filed January 7, 1922. Serial No. 527,726.

*To all whom it may concern:*

Be it known that I, JOHN C. BAKER, a citizen of the United States of America, residing at Nutley, Essex County, State of New Jersey, have invented certain new and useful Improvements in Bleaching Paper Pulp, of which the following is a full, clear, and exact description.

The process of bleaching paper pulp has heretofore been carried out almost universally by the use of a sufficient amount of a solution of bleaching powder which is added to the unbleached pulp. Under ordinary conditions the bleaching action is continued until its completion, which requires from three to six hours, but at or before the expiration of this period it is customary to add an acid to improve the final bleaching effect. This addition of acid, however, is usually ineffective in producing the desired result, and, in fact, is frequently disadvantageous by increasing instead of diminishing the color of the pulp and thus actually impairing, rather than improving, the intended bleaching action.

By a protracted course of experiment and investigation I have ascertained the reason for the unsatisfactory colors in such product as wood pulp, and have discovered a new method for very greatly increasing the whiteness of the finished stock without in any way impairing its properties, and this application for Letters Patent is based upon that discovery, which I shall now describe in detail.

I have found that there may exist two differently acting coloring matters which are left in the nearly bleached pulp. One of these is the principal coloring matter of the pulp which remains as the result of incomplete bleaching, but which is capable of being eliminated by the continued bleaching action, and the other is a color which cannot be eliminated by further bleaching nor entirely by the usual step of adding an acid.

When this first-named or unbleached color remains in the pulp the addition of acid results in the liberation of chlorine from remaining bleach which attacks the color and forms fixed yellows which cannot be then removed, and this is the main cause of the retrogression following the addition of acid. On the other hand, the other coloring matter present in the pulp is not affected by the use of acid as ordinarily practiced

for reasons which will be explained, although, if a great excess of acid is added, or if the pulp be washed and then acidified, or if acid be added and the pulp be allowed to stand for a long period, as, for example, over night, then the pulp becomes very white.

These methods are not, however, practicable nor feasible because of the impairment by their use of the fibre strength, or because of the increase of time involved or the expense and complication of the washing equipment required for the proper removal of the acid.

I have found that the color may be eliminated and color retrogression effectively prevented if the residual available chlorine, which remains at the point of complete bleaching action is destroyed by a reducing agent, and the acid then either simultaneously or subsequently added.

The reasons for these steps will be understood from the following:



in which  $\text{CaOCl}_2$  is calcium hypochlorite, and  $\text{HOCl}$  is hypochlorous acid. The hypochlorous acid formed is a very weak acid and is not sufficiently ionized to yield hydrogen ions which are capable of changing the coloring matter in the pulp. The addition of acid is, therefore, without sensible effect. The addition of stronger acid beyond that required to react with all of the calcium hypochlorite results in some improvement in the color, but a rather large amount is required for the optimum effect. This is due to the presence of the oxidizing potential of the hypochlorous acid, which appears to hold the color in a condition in which it is not readily changed by acid. But, if all the available chlorine is destroyed, a relatively small amount of acid is all sufficient to produce the desired result.

The addition of more reducing agent beyond that required to destroy the hypochlorite, produces a further whitening effect on the pulp in the presence of the added acid.

In the carrying out of my new process, there are many agents which can be used such as hyposulphite of sulphites with sulphuric acid or oxalic acid alone, but for economy of operation and for obtaining the most satisfactory results, the most desirable agent is sulphur dioxide, as this operates both as a reducing and as an acidifying agent, and

may be used in amounts in excess of that required for destroying the hypochlorite without damage or injury, and will further improve the color. Other acids may be used 5 with the sulphur dioxide, if sufficient be not employed for the complete destruction of the hypochlorite, to produce the desired results.

The reactions occurring in the process may be thus expressed:



or in other words, calcium hypochlorite plus sulphur dioxide plus water gives calcium chloride plus sulphuric acid.

15 This removes the oxidizing potential and adds acid at the same time. A further reaction can occur with the color when more  $\text{SO}_2$  is added which results in additional color removal.

20 I have herein described the application of the process, the ordinary and well known bleaching process, but its use is not limited in this respect. For example, I may use it in conjunction with a process of my invention which I have set forth in an application Serial No. 485,701, filed July 18, 1921.

Having now described my invention, what I claim is:—

1. The process of bleaching pulp by an agent containing chlorine herein described, 30 which consists in continuing the process until the bleaching effect is practically complete, then neutralizing or destroying in the pulp the remaining chlorine component and acidifying the pulp. 35

2. The process of bleaching pulp herein described which consists in exposing the pulp to the action of a bleaching agent containing chlorine until the bleaching effect is practically complete, then adding an 40 agent to destroy the remaining chlorine and then adding an acid. 45

3. The process of bleaching pulp herein described which consists in exposing the pulp to the action of a bleaching agent containing chlorine until the bleaching effect is practically complete, and then adding sulphur dioxide.

In testimony whereof I hereto affix my signature.

JOHN C. BAKER.

CERTIFICATE OF CORRECTION.

Patent No. 1,468,693.

September 25, 1923.

JOHN C. BAKER.

It is hereby certified that error appears in the printed specification of the above numbered patent requiring correction as follows: Page 1, second column, line 107, for the word "of" read --or--; and that the said Letters Patent should be read with this correction therein that the same may conform to the record of the case in the Patent Office.

Signed and sealed this 30th day of July, A. D. 1940.

Henry Van Arsdale,  
Acting Commissioner of Patents.

(Seal)